

## UNITED STATES PATENT OFFICE

2,496,903

PHOTOGRAPHIC DEVELOPER CONTAINING  
A NEGATIVELY SUBSTITUTED ARALKYL-  
AMINE AND PROCESS OF DEVELOPMENTWilliam L. Wasley, Binghamton, N. Y., assignor to  
General Aniline & Film Corporation, New York,  
N. Y., a corporation of DelawareNo Drawing. Application November 18, 1947,  
Serial No. 786,816

12 Claims. (Cl. 95—88)

1

This invention relates to photographic developers and particularly to accelerators for photographic developers.

It is well-known that various amines, such as primary and secondary alkyl and alkylene amines containing from 3 to 7 carbon atoms, and heterocyclic amines such as morpholine and piperidine as disclosed in United States Patent 2,304,025, may be added to photographic black and white and color developing solutions for the purpose of increasing the rate of development. In other words, these amines accelerate the development so as to cause the developing agent to form the image (silver or color image) more rapidly than is possible without the presence of such amines.

Although developing solutions containing such amines cut the developing time from about 20 to 30 minutes to 12 to 15 minutes, such a decrease is still unsatisfactory where large scale operations are involved, as in commercial processing where time is of the essence.

It is also known that there are aralkylamines which, when present in developing solutions in an amount ranging from 8 to 30 cc. per liter, energize weak developers to the extent that second exposure is not necessary for reversal development.

It has always been assumed by the art, however, that these aralkyl amines, in order to be operative as energizers for developing solutions, must be free from negative groups such as nitro, hydroxy, sulfonic acid, halogen atoms, e. g., Cl, Br, and the like. It has now been found that certain aralkyl amines in which negative groups such as nitro, and halogen atoms are attached to a carbon atom in the aryl ring greatly accelerate development rates and energize weak developers to an extent that no second exposure is necessary for reversal development. This discovery is wholly surprising and unexpected in view of the contrary teachings and assumption by those skilled in the art.

It is, therefore, an object of the present invention to provide a black and white and color developer having an increased rate of development so that the developing time is substantially decreased to about one-half of the normal time.

Other objects will appear hereinafter.

These objects are accomplished by adding an aralkylamine containing a negative nitro or halogen group attached to a carbon in the aryl ring to the usual black and white developer, and to a color-forming developer in which a primary aromatic amine is used as the developing agent. It has been found that in develop-

2

ing color images in multi-color photographic layers containing color-formers fast to diffusion, as disclosed in United States Patents 2,178,612; 2,179,228; 2,179,234; 2,179,238-9; 2,179,244; 2,186,719; 2,186,851-2; 2,186,732-3-4; 2,186,849; 2,200,306; 2,280,722; 2,292,575; 2,303,928 and 2,307,399, with a color developer containing a negatively substituted aralkyl amine, the developing time is cut from 20-30 minutes to 2-10 minutes. All of the layers are simultaneously developed, and the dye images formed are of excellent quality.

The developing time with black and white developers, for instance, solutions of hydroquinone and monomethylamine-m-phenol sulfate and the like, is also cut to about one-half without causing fog when such solutions contain a negatively substituted aralkylamine.

The negatively substituted aralkylamines to be employed in accordance with the present invention are represented by the following general formulae:



and



35

wherein R is methyl or ethyl, n is a positive integer of from 1 to 2, and X is a negative group such as nitro, chlorine, bromine and the like.

The following are examples of such negatively substituted aralkyl amines:



p-chlorobenzylamine



m-bromobenzylamine



## 3

p-nitrobenzylamine

 $\alpha$ -[p-chlorophenyl]-ethylamine $\alpha$ -[p-chlorophenyl]-propylamine $\beta$ -[m-bromophenyl]-ethylamine

These amines possess limited solubility in water and in alkaline developers. Their solubility in water and in alkaline developers, however, is made appreciable by converting the base into a salt such as, for example, the hydrochloride or carbonate. The hydrochloride salt is readily prepared by the addition of a stoichiometrical quantity of hydrochloric acid, and the carbonate is prepared by bubbling  $\text{CO}_2$  into an alcohol, ether or benzene solution of the base. The most useful concentrations in black and white and color developers range from about 1 to 7 grams per liter of developer solution.

As illustrative developing solutions containing such aralkylamines, the following are given:

## Example I

|                                    | Grams |
|------------------------------------|-------|
| p-Monomethylamine-m-phenol sulfate | 0.8   |
| Sodium sulfite (anhydrous)         | 45    |
| Hydroquinone                       | 1.2   |
| Sodium carbonate (monohydrate)     | 8     |
| Potassium metabisulfite            | 4     |
| Potassium bromide                  | 1.5   |
| p-Chlorobenzylamine                | 4     |
| Water to make liter                | 1     |

This tank developer gives, on development at 20° C. of the usual roll film, a soft negative in about 6-10 minutes after fixing and washing. The time required to develop a similar roll in the same developer and at the same temperature, but containing no p-chlorobenzylamine, ranges from 15 to 20 minutes. Increasing the concentration of the p-chlorobenzylamine to 7 grams per liter effects a further decrease in time.

## Example II

The following developer requires 30 minutes at 20° C. to give a satisfactory degree of color development with color paper:

|                                                                 | Grams |
|-----------------------------------------------------------------|-------|
| Sodium hexametaphosphate                                        | 1.0   |
| Sodium bisulfite                                                | 2.0   |
| N - N - bis( $\beta$ -hydroxyethyl)-p-phenylene-diamine sulfate | 6.3   |
| Sodium carbonate                                                | 100   |
| Hydroxylamine hydrochloride                                     | 1.0   |
| Potassium bromide                                               | 1.0   |
| Water to make liter                                             | 1     |

## 4

By the addition of 5 grams of  $\alpha$ -(p-chlorophenyl)-ethylamine to the foregoing developing solution, a color paper of excellent color rendition is developed in 10 minutes. Increasing the concentration of the amine further reduces the time of development.

The color paper (photographic multi-layer element) utilized in the foregoing example, consists of an integral tripack emulsion coated on either the usual paper base, or a clear cellulose acetate or nitrate film base, or in some cases an opaque white film base. Each of the emulsion layers is sensitized to one of the primary colors of light; namely, blue, green and red. The top layer is blue sensitive. A filter layer, yellow in color and blue absorbing, lies under the top layer. Below this filter layer, lies a green sensitive emulsion layer, and below this a red sensitive emulsion layer. Each of the three silver-halide emulsion layers contains dye-forming compounds which unite during the development of a silver image in an aromatic amine developing agent to form a dye with the oxidation product of the developing agent. As silver is also formed during development, it must be removed after color development by treatment in a bleach, followed by a bath of sodium thiosulfate, as is well-known to the art. A yellow dye is formed in the blue sensitive emulsion; a magenta dye is formed in the green sensitive emulsion; and a cyan dye is formed in the red sensitive emulsion. The combination of the dye images from these three printing primaries yields the color picture. Suitable methods for the preparation of multi-color emulsion layers have been described in the literature relating to color photography, and are, therefore, not described here.

## Example III

The following developer requires 19 minutes at 20° C. to give a satisfactory degree of color development with color paper:

|                                                        | Grams |
|--------------------------------------------------------|-------|
| Sodium hexametaphosphate                               | 1.0   |
| Sodium bisulfite                                       | 2.0   |
| N - ethyl - N-hydroxyethyl-p-phenylene-diamine sulfate | 6.7   |
| Sodium carbonate                                       | 100   |
| Hydroxylamine hydrochloride                            | 1.0   |
| Potassium bromide                                      | 1.0   |
| Water to make liter                                    | 1     |

By the addition of 3.5 grams of p-nitrobenzylamine to the foregoing developing solution, a color paper of excellent color rendition is developed in 10 minutes. Increasing the concentration of the amine to 6 grams reduces the time of development to 6 minutes with the same results.

## Example IV

The color developer of the preceding example with the addition of 5 grams of p-chlorobenzylamine developed a multi-layer color film sheet, of the reversal type, and containing color-formers fast to diffusion, in 10 minutes at 20° C., whereas without the p-chlorobenzylamine, the time required to color develop the said film sheet is over 30 minutes.

What I claim is:

- An alkaline photographic developer for silver-halide comprising a silver-halide developer and a negatively substituted aralkylamine select-

ed from the class consisting of those corresponding to the following formulae:



and



wherein R is a group selected from the class consisting of methyl and ethyl groups, n is a positive integer of from 1 to 2, and X is a negative group selected from the class consisting of nitro and halogen atoms, and the salts of said amines.

2. An alkaline photographic developer for silver-halide comprising a silver-halide developer and a negatively substituted aralkylamine characterized by the following formula:



3. An alkaline photographic developer for silver-halide comprising a silver-halide developer and a negatively substituted aralkylamine characterized by the following formula:



4. An alkaline photographic developer for silver-halide comprising a silver-halide developer and a negatively substituted aralkylamine characterized by the following formula:



5. In the development of a photographic negative the step comprising the development of an exposed silver-halide emulsion in an alkaline developer containing a developing agent for said emulsion and a developing accelerator selected from the class consisting of negatively substituted aralkyl amines corresponding to the following formulae:



and



wherein R is a group selected from the class consisting of methyl and ethyl groups, n is a positive integer of from 1 to 2, and X is a negative group selected from the class consisting of nitro and halogen atoms, and the salts of said amines.

6. In the development of a photographic negative the step comprising the development of an

exposed silver-halide emulsion in an alkaline developer containing a developing agent for said emulsion and a developing accelerator characterized by the formula:



10 7. In the development of a photographic negative the step comprising the development of an exposed silver-halide emulsion in an alkaline developer containing a developing agent for said emulsion and a developing accelerator characterized by the formula:



20 8. In the development of a photographic negative the step comprising the development of an exposed silver-halide emulsion in an alkaline developer containing a developing agent for said emulsion and a developing accelerator characterized by the formula:



25 9. A color-forming photographic developer comprising a primary aromatic amino developing agent and a negatively substituted aralkylamine selected from the class consisting of those corresponding to the following formulae:



and



50 wherein R is a group selected from the class consisting of methyl and ethyl groups, n is a positive integer of from 1 to 2, and X is a negative group selected from the class consisting of nitro and halogen atoms, and the salts of said amines.

55 10. A color-forming photographic developer comprising a primary aromatic amino developing agent and a negatively substituted aralkylamine characterized by the following formula:



60 11. A color-forming photographic developer comprising a primary aromatic amino developing agent and a negatively substituted aralkylamine characterized by the following formula:



12. A color-forming photographic developer comprising a primary aromatic amino developing agent and a negatively substituted aralkyl-amine characterized by the following formula:



WILLIAM L. WASLEY.

**REFERENCES CITED**

The following references are of record in the file of this patent:

**UNITED STATES PATENTS**

| Number    | Name          | Date         |
|-----------|---------------|--------------|
| 2,410,644 | Fierke et al. | Nov. 5, 1946 |